# EUROPEAN PATENT SPECIFICATION

(11) **EP 0 750 033 B1**
(45) Date of publication and mention of the grant of the patent: **22.03.2000**
(21) Application number: 96304602.4
(22) Date of filing: 20.06.1996
(51) Int. Cl.: C10M 169/04

(54) **Hydraulic fluid composition**
Hydraulische Flüssigkeitzusammensetzung
Composition de fluide hydraulique

(30) Priority: 23.06.1995 FR 9507955
(43) Date of publication of application: 27.12.1996
(73) Proprietor: BP Chemicals Limited, London EC2M 7BA (GB); BP CHEMICALS S.N.C., 92400 Courbevoie (FR)
(72) Inventor: Broussard, Christian, BP No. 6, 13117 Lavera (FR); Decroocq, Serge, BP No. 6, 13117 Lavera (FR)
(74) Representative: Hymers, Ronald Robson

(56) References cited:
- GB-A- 908 291
- GB-A- 1 131 263
- US-A- 2 580 036
- US-A- 3 003 968
- US-A- 3 206 486
- US-A- 3 784 474
- US-A- 3 914 182
- US-A- 4 371 448
- US-A- 5 204 012

## Description

The present invention relates to a hydraulic fluid composition, especially a brake fluid composition employed in particular in the braking systems of motor vehicles, and to a process for the treatment of a hydraulic fluid with a view to reducing the corrosion of the ferrous alloys or metals in contact with the said fluid.

US Patent No. 3,914,182 discloses a hydraulic fluid composition comprising a borate ester of a glycol ether and an ester or a mixture of esters selected amongst esters of formula (I) and (II). The ester of formula (I) is a dicarboxylic acid ester, and the ester of formula (II) is a C₂ or C₃ carboxylic acid di-ester of glycol. Furthermore the composition may comprise various additives selected amongst lubricity additives, antioxidants, corrosion inhibitors and stabilizers such as primary or secondary aliphatic amines containing from 4 to 12 carbon atoms.

US Patents No. 2,580,036, No. 5,204,102 and No. 3,784,474 disclose mineral lubricating oil compositions essentially comprising a base oil which exhibits hydrophobic and film-forming properties.

US Patent No. 3,003,968 discloses a hydraulic fluid composition comprising a C₂ to C₅ carboxylic acid di-ester of polyoxyethylene glycols.

GB Patent Application No. 1,131,263 discloses a hydraulic fluid composition based on glycol ether or a mixture of a polyalkylene glycol and a glycol ether. The composition is not based on a boric ester of a glycol ether.

GB Patent Application No. 908,291 discloses esters of ricinoleic acid and polyalkylene glycols which are particularly useful as constituents of hydraulic fluid composition. However the composition is not based on a boric ester of a glycol ether.

US Patent No. 3,206,486 discloses fatty acid monoesters of polyoxypropylene-polyoxyethylene block copolymer glycols and their use in brake fluid compositions. However, the compositions are not based on a boric ester of a glycol ether.

There is a hydraulic fluid composition which is known, especially according to US Patent No. 4,371,448, essentially based on a boric ester of a glycol ether and comprising an alkylamine optionally with corrosion-inhibiting agent chosen from fatty acids, esters of phosphorous or phosphoric acid with a C₁-C₆ aliphatic alcohol and triazoles.

However, the known brake fluid compositions still leave something to be desired. The reason for this is, above all, that amongst the requirements which a brake fluid composition should fulfil, there are also those which are conflicting because of the chemical and physical properties of the main components. Thus, for example, it is known to be very difficult to adjust the viscosity of a brake fluid composition based on a boric acid esters in accordance with the DOT-5.1 standard and at the same time also to achieve an excellent corrosion inhibiting system. When formulating known brake fluid compositions based on boric acid esters, a gain in an important property is thus frequently brought by a relatively high sacrifice in another important property. Furthermore, what is known in a lubricating oil composition having hydrophobic and film-forming properties cannot be applied to a boric acid ester composition for hydraulic fluid composition having hydrophilic and hygroscopic properties, since the corrosion mechanismes are different.

It has been observed that the hydraulic fluid compositions known hitherto, like that mentioned above, do not simultaneously satisfy a number of requirements such as extremely high boiling points, a low kinematic viscosity at low temperature and a high protection against corrosion of ferrous alloys or metals, especially in a moist atmosphere. In particular, some manufacturers and/or users of motor vehicles such as military vehicles now demand that the brake fluid compositions should be capable of simultaneously satisfying the following characteristics :
- a dry boiling point of at least 260°C and a wet boiling point of at least 180°C, as defined in the US Department of Transportation standard DOT 5.1,
- a kinematic viscosity at - 40°C of not more than 1500 mm²/s, as defined in ISO standard 4925, and
- an excellent protection against the corrosion of ferrous alloys or metals in a moist atmosphere, especially when it is known that some water uptake by brake fluids may appear after a long period of nonutilization of the vehicles.

A hydraulic fluid composition has now been found, and especially a brake fluid composition based essentially on a boric ester of a glycol ether comprising a corrosion-inhibitor system, allowing the abovementioned requirements to be satisfied simultaneously. The composition and in particular its corrosion-inhibiting system, must ensure at the same time good compatibility with water originating a possible water uptake of the composition and excellent anticorrosive properties in a moist atmosphere, while maintaining the boiling point and kinematic viscosity characteristics, especially at the very severe levels demanded by the abovementioned standards.

The present invention therefore relates to a hydraulic fluid composition based essentially on a boric ester of a glycol ether, comprising a corrosion-inhibiting system, characterized in that it includes :
(1) at least one constituent (A) chosen from fatty, and optionally ethoxylated, mono-, di- or polyamines, said fatty amines containing at least one C₈-C₂₂ alkyl or alkylene radical R, the alkylene radical R may contain one or more ethylenic double bond or from the salts of one or more carboxylic acids with the said amines, in an amount of 0.05 to 2% by weight of the constituent(s) (A), and
(2) at least one constituent (B) chosen from the products resulting from the reaction of one or more carboxylic fatty acids with a polyoxyalkylene glycol or from the transesterification reaction of one or more esters of carboxylic fatty acids with a polyoxyalkylene glycol, in an amount of 0.5 to 10% by weight of the constituent(s) by said fatty acids being monocarboxylic acids with 8 to 22 carbon atoms.

Fatty mono-, di- or polyamines mean primary, secondary or tertiary amines containing at least one C₈-C₂₂, preferably C₁₃-C₂₂, especially C₁₅-C₁₈, e.g. C₁₆ or C₁₈ alkyl or alkylene radical R, the alkylene radical R which may contain one or more ethylenic double bonds.

The constituent (A) may be especially a fatty mono-, di- or polyamine corresponding to one of the following general formulae : ${\text{R}}^{\text{1}} {\text{- NH - (CH}}_{\text{2}} {\text{)}}_{\text{3}} {\text{- NH}}_{\text{2}} {\text{; R}}^{\text{1}} {\text{- [NH - (CH}}_{\text{2}} {\text{)}}_{\text{3}} {\text{]}}_{\text{2}} {\text{- NH}}_{\text{2}} \text{;} {\text{R}}^{\text{1}} {\text{- [NH - (CH}}_{\text{2}} {\text{)}}_{\text{3}} {\text{]}}_{\text{n}} {\text{- NH}}_{\text{2}} \text{;}$ in which general formulae R¹ and R², being identical or different, have the definition of the abovementioned radical R, n is a number ranging from 3 to 6, and x, y and z, being identical or different, are numbers ranging from 1 to 3.

The constituent (A) is preferably the salt of one or more carboxylic fatty acids, especially C₈-C₂₂, with one of the fatty mono-, di- or polyamines corresponding especially to one of the preceding general formulae and in particular to the general formula :

R¹-NH-(CH₂)₃-NH₂

in which R¹ has the same definition as above.

Also the constituent (A) is preferably a fatty diamine, in particular corresponding to general formula :

R¹-NH-(CH₂)₃-NH₂

in which R¹ has the same definition as above, in particular R¹ is an alkylene radical, e.g. a C₁₈ alkylene radical.

The constituent (B) may be the product of the reaction of one or more carboxylic fatty acids, especially C₈-C₂₂, with a polyoxyalkylene glycol such as diethylene glycol or preferably dipropylene glycol. It may also be the product of the transesterification reaction of one or more esters of carboxylic fatty acids, especially C₈-C₂₂, preferably of one or more glycerides of the said carboxylic fatty acids, with a polyoxyalkylene glycol such as diethylene glycol or preferably dipropylene glycol. The constituent (B) may be preferably the product of the transesterification reaction of castor oil with a polyoxyalkylene glycol such as diethylene glycol or especially dipropylene glycol. The polyoxyalkylene glycol involved in the above-mentioned reaction products used as constituent (B) generally corresponds to the general formula :

HO- (CH₂ CHR²O)ₙ - H

in which R² represents a hydrogen atom or a C₁ - C₄ alkyl radical, preferably the methyl radical, and n is a number ranging from 1 to 4, preferably equal to 2 or 3, especially equal to 2.

Fatty acids are monocarboxylic acids with 8 to 22, preferably 12 to 20, especially 15 to 18, e.g. 18 carbon atoms.

The composition according to the invention includes from 0.05 to 2 %, preferably from 0.1 to 1 % by weight of the constituent(s) (A) and from 0.5 to 10 %, preferably from 1 to 8 % by weight of the constituent(s) (B).

The composition is based essentially on a boric ester of a glycol ether in a proportion that can range from 40 to 95 %, preferably from 65 to 95 % by weight. The boric ester of a glycol ether preferably is a boric ester of an ethylene glycol monoalkyl ether which is generally obtained when reacting orthoboric acid and an ethylene glycol monoalkyl ether corresponding to the formula :

R³ (OCH₂ CH₂)ₘ OH

in which R³ represents an alkyl radical e.g. with 1 to 4, preferably 1 or 2 carbon atoms, and m is a number ranging from 1 to 4, preferably 2 to 3. The preferred boric ester of a glycol ether is the boric ester of triethylene glycol monomethyl ether. The composition may additionally advantageously include at least one glycol ether such as triethylene glycol monobutyl ether or monoethyl ether or, preferably, triethylene glycol monomethyl ether in a proportion that can range from 5 to 40 %, preferably from 10 to 30 % by weight.

The composition may also include other additives such as corrosion-inhibiting agents. In particular it may include the following additives :
- from 0.5 to 5 % by weight of at least one amine capable especially of neutralizing the boric ester employed, in particular an amine containing at least one alkyl radical, especially from C₁ to C₇, or a cyclane radical, especially from C₅ to C₇, or, again, an alkoxy radical especially from C₁ to C₆, or one of these ethoxylated amines, for example di-n-butylamine, tri-n-butylamine, diisopropanolamine of general formula : HN(CH₂ CHOHCH₃)₂, monocyclohexylamine, dicyclohexylamine, 2-amino-1-ethanol, diethanolamine of general formula : HN (CH₂ - CH₂ OH)₂, monomethanolmonopropylamine of general formula : HN (CH₂OH) (CH₂ CH₂ CH₃) or diisopropylamine ;
- from 0.1 to 2 % by weight of an N-acyl derivative of sarcosine, for example the N-oleyl acylsarcosine marketed by Ciba Geigy under the name « Sarkosyl 0 » ®
- from 0.1 to 2 % by weight of corrosion-inhibiting additives such as benzotriazole or tolyltriazole, triphenyl phosphite, dodecenylsuccinic anhydride or an antioxydant such as bisphenol A or polymerized trimethylquinoline.

All the percentages by weight given in each case above relate to the total weight of the composition and so that the sum of the percentages of the composition is always equal to 100.

The composition according to the present invention may be prepared by mixing the constituents (A) and (B) and optionally other constituents and additives with the boric ester of a glycol ether, in any order, under an inert atmosphere such as nitrogen, and at a temperature that can range from - 20 to + 50°C.

The hydraulic fluid composition according to the present invention is particularly suitable for being employed as brake fluid. It may additionally satisfy the requirements of the standards FMVSS 116-DOT 4 and in particular of the standards DOT 5.1 relating to the dry and wet boiling points, the requirements of the ISO standard 4925 relating to kinematic viscosity at - 40°C and those of the SAE standard J 1703 - January 1995, relating to the fluidity and the appearance of the brake fluid at - 50°C, and may simultaneously exhibit excellent anticorrosive properties in a moist atmosphere according to the LCSEA-C-6 test method of the French Armies' Department of Petrols.

The present invention also relates to a process for the treatment of a hydraulic fluid composition, especially of a brake fluid composition including a boric ester of a glycol ether, preferably the boric ester of triethylene glycol monomethyl ether, and optionally a glycol ether such as triethylene glycol monobutyl ether or monoethyl ether or preferably triethylene glycol monomethyl ether, a treatment for reducing the corrosion of ferrous alloys or metals in contact with the said composition, especially in a moist atmosphere, including the addition of a corrosion-inhibiting system, characterized in that the corrosion-inhibiting system includes :
(1) at least one constituent (A) chosen from fatty and optionally ethoxylated mono-, di- or polyamines, or from the salts of one or more carboxylic acids with the said amines, in an amount of 0.05 to 2% by weight of the constituent(s) (A), and
(2) at least one constituent (B) chosen from the products resulting from the reaction of one or more carboxylic fatty acids with a polyoxyalkylene glycol, or from the transesterification reaction of one or more esters of carboxylic fatty acids with a polyoxyalkylene glycol, in an amount of 0.5 to 10% by weight of the constituent(s) (B).

In particular, the constituents (A) an (B) may correspond to those described above and especially to the preferred constituents (A) and (B), employed in particular in the abovementioned proportions. The composition treated according to the present invention may additionally include additives such as those mentioned above and in the same proportions. The present process for treatment of a hydraulic fluid composition, in particular of brake fluid, has the advantage of ensuring an excellent protection against the corrosion of ferrous alloys or metals especially in a humid atmosphere, while maintaining the dry and wet boiling points and the kinematic viscosity at - 40°C at the level of the abovementioned standards, without causing turbidity or crystallization at - 50°C under a moist atmosphere.

In the process of the invention the constituents (A) and (B) and optionally other constituents or additives may be mixed with the boric ester of a glycol ether in any order, under an inert atmosphere such as nitrogen and a temperature that can range from - 20° to + 50°C.

### Test and measurement methods :

- the dry boiling point, or equilibrium reflux boiling point (ERBP), is measured in °C according to the ASTM method D-1120 ;
- the wet equilibrium reflux boiling point (WERBP) is measured in °C according to the method of the SAE standard J 1703 - January 1995 ;
- the fluidity and the appearance at - 50°C are measured and assessed according to the methods of the SAE standard J 1703 - January 1995 ;
- the anticorrosive properties in a moist atmosphere are measured according to the method LC SEA-C-6 of the French Armies' Department of Petrols, a method which includes :
   to N-oleyl of sarcosine, as additive,
- « Duomeen 0 » ® marketed by the company Akzo Nobel, corresponding to N-oleyl-1,3-diaminopropane, as constituent (A),
- « Inipol 002 » ® marketed by the company CECA, corresponding to N-oleyl-1,3-diaminopropane dioleate, as constituent (A),
- « Delco A Base » ® manufactured by BP Chemicals, corresponding to the ester obtained by transesterification of castor oil with dipropylene glycol, as constituent (B).

### Comparative tests 1 to 4 and Example 5

Brake fluid comparative compositions 1 to 4 and the brake fluid composition 5 according to the present invention are prepared by mixing the various constituents mentioned in Table 1 at ambient temperature (20°C) and under a nitrogen atmosphere.

The results of the measurements and tests performed on these compositions are collated in Table 2.

Analysis of Tables 1 and 2 shows that :
- only composition 5 according to the present invention, including especially 0.4 % by weight of « Inopol 002 » ® as constituent (A) and 4 % by weight of « Delco A Base » ® as constituent (B) makes it possible simultaneously to satisfy all the requirements of the abovementioned standards and to exhibit excellent anticorrosive properties in a moist atmosphere ;
- although the comparative compositions 1 to 3 contain the constituent (A) in proportions (0.5 %, 1.0 %, 1.0 % by weight respectively) which are higher than that in composition 5 (0.4 % by weight), and although comparative composition 4 contains the constituent (B) in a proportion (10.0 % by weight) which is much higher than that in composition 5 (4.0 % by weight), none of these comparative compositions exhibits satisfactory anticorrosive properties in a moist atmosphere, nor do they satisfy simultaneously all the requirements of dry or wet boiling point, of kinematic viscosity at - 40°C and of appearance at - 50°C.

The constituents (A) and (B) employed simultaneously in the present invention form, through a synergy effect, a hydraulic fluid and especially brake fluid composition with excellent properties which are superior of those of the comparative compositions containing only a single one of the constituents (A) and (B), even in proportions that are very markedly high than those employed in the present composition.

### Example 6

Brake fluid composition 6 according to the present invention is prepared by mixing the following various constituents at ambient temperature (20°C) and under a nitrogen atmosphere :
% by weight
- boric ester of triethylene glycol monomethyl ether : 72.0
- triethylene glycol monomethyl ether : 19.9
- cyclo-hexylamine : 1.0
- other specific additives (see (1) in Table 1) : 2.1
- « Sarkosyl 0 » ®: 0.5
- « Duomeen 0 » ® [constituent (A)] : 0.5
- « Delco A Base » ® [constituent (B)] : 4.0

The results of the measurements and tests performed on this composition are collected hereafter :
- ERBP : 265°C
- WERBP : 182°C
- kinematic viscosity at - 40°C : 1350 mm²/s
- fluidity and appearance at - 50°C :
   . appearance : bright and clear
   . flow time : 6 s
- test for corrosion in moist atmosphere :
   . corrosion spots : 0
   . comments : very satisfactory.

## Claims

1. Hydraulic fluid composition based essentially on a boric ester of a glycol ether, comprising a corrosion-inhibiting system, characterized in that it includes :
(1) at least one constituent (A) chosen from fatty, and optionally ethoxylated, mono-, di- or polyamines, said fatty amines containing at least one C₈-C₂₂ alkyl or alkylene radical R, the alkylene radical R may contain one or more ethylenic double bond, or from the salts of one or more carboxylic acids with the said amines, in an amount of 0.05 to 2% by weight of the constituent(s) (A), and
(2) at least one constituent (B) chosen from the products resulting from the reaction of one or more carboxylic fatty acids with a polyoxyalkylene glycol or from the transesterification reaction of one or more esters of carboxylic fatty acids with a polyoxyalkylene glycol, in an amount of 0.5 to 10% by weight of the constituent(s) (B), said fatty acids being monocarboxylic acids with 8 to 22 carbon atoms.

2. Composition according to Claim 1, characterized in that the constituent (A) is a fatty mono-, di- or polyamine corresponding to one of the following general formulae : ${\text{R}}^{\text{1}} {\text{- NH - (CH}}_{\text{2}} {\text{)}}_{\text{3}} {\text{- NH}}_{\text{2}} {\text{; R}}^{\text{1}} {\text{- [NH - (CH}}_{\text{2}} {\text{)}}_{\text{3}} {\text{]}}_{\text{2}} {\text{- NH}}_{\text{2}} \text{;} {\text{R}}^{\text{1}} {\text{- [NH - (CH}}_{\text{2}} {\text{)}}_{\text{3}} {\text{]}}_{\text{n}} {\text{- NH}}_{\text{2}} \text{;}$ in which general formulae R¹ and R², being identical or different, denote a C₈-C₂₂ alkyl or alkylene radical R, the alkylene radical R containing 1 or more ethylenic double bonds, n is a number ranging from 3 to 6, and x, y and z, being identical or different, are numbers ranging from 1 to 3.

3. Composition according to Claim 1 to 2, characterized in that the constituent (A) is the salt of one or more carboxylic fatty acids with one of the fatty mono-, di- or polyamines.

4. Composition according to Claim 3, characterized in that the fatty mono- di- or polyamine corresponds to the general formula
R¹ - NH - (CH₂)₃ - NH₂
in which R¹ denotes a C₈-C₂₂ alkyl or alkylene radical R, the alkylene radical R containing one or more ethylenic double bonds.

5. Composition according to any one of Claims 1 to 4, characterized in that the constituent (B) is the product resulting from the reaction of one or more C₈-C₂₂ carboxylic fatty acids with diethylene glycol or dipropylene glycol or from the transesterification reaction of one or more glycerides of C₈-C₂₂ carboxylic fatty acids with diethylene glycol or dipropylene glycol.

6. Composition according to any one of Claims 1 to 5, characterized in that the constituent (B) is the product of the transesterification reaction of castor oil with diethylene glycol or dipropylene glycol.

7. Composition according to any one of Claims 1 to 6, characterized in that it includes from 0.1 to 1 % by weight of the constituent(s) (A) and from 1 to 8 % by weight of the constituent(s) (B).

8. Composition according to any one of Claims 1 to 7, characterized in that it is based essentially on the boric ester of triethylene glycol monomethyl ether and optionally comprised a glycol ether chosen from triethylene glycol monobutyl ether or monoethyl ether or monomethyl ether.

9. Process for the preparation of the composition according to any one of Claims 1 to 8, characterized in that the constituents (A) and (B) and optionally other constituents and additives are mixed with the boric ester of a glycol ether under an inert atmosphere.

10. Process for the treatment of a hydraulic fluid composition including a boric ester of a glycol ether, in order to reduce the corrosion of ferrous alloys or metals in contact with the said composition, including the addition of a corrosion-inhibiting system, characterized in that the corrosion-inhibiting system includes :
(1) at least one constituent (A) chosen from fatty, and optionally ethoxylated, mono-, di- or polyamines, said fatty amines containing at least one C₈-C₂₂ alkyl or alkylene radical R, the alkylene radical R may contain one or more ethylenic double bond, or from the salts or one or more carboxylic acids with the said amines, in an amount of 0.05 to 2% by weight of the constituent(s) (A), and
(2) at least one constituent (B) chosen from the products resulting from the reaction of one or more carboxylic fatty acids with a polyoxyalkylene glycol or from the transesterification reaction of one or more esters of carboxylic fatty acids with polyoxyalkylene glycol, in an amount of 0.5 to 10% by weight of the constituent(s) (B), said fatty acids being monocarboxylic acids with 8 to 22 carbon atoms.

## Patentansprüche

1. Hydraulische Flüssigkeitzusammensetzung, basierend im wesentlichen auf einem Borsäureester eines Glykolethers, enthaltend ein korrosionsinhibierendes System, dadurch gekennzeichnet, daß es einschließt:
(1) Zumindest einen Bestandteil (A), ausgewählt aus fettigen und wahlweise ethoxylierten, Mono-, Di- oder Polyaminen, und Fettaminen, enthaltend zumindest einen C₈₋₂₂-Alkyl- oder -Alkylenrest R, wobei der Alkylenrest R eine oder mehrere ethylenische Doppelbindungen enthalten kann, oder aus den Salzen von einer oder mehreren Carbonsäuren mit den erwähnten Aminen in einer Menge von 0,05 bis 2 Gew.-% des Bestandteils (der Bestandteile) (A), und
(2) zumindest einen Bestandteil (B), ausgewählt aus den Produkten, resultierend aus der Reaktion von einer oder mehreren Carbonfettsäuren mit einem Polyoxyalkylenglykol, oder aus der Umesterungsreaktion von einem oder mehreren Estern von Carbonfettsäuren mit einem Polyoxyalkylenglykol in einer Menge von 0,5 bis 10 Gew.-% des Bestandteils (der Bestandteile) (B), wobei die erwähnten Fettsäuren Monocarbonsäuren mit 8 bis 22 Kohlenstoffatomen sind.

2. Zusammensetzung nach Anspruch 1, dadurch gekennzeichnet, daß der Bestandteil (A) ein Fett-mono-, -di- oder -polyamin ist, entsprechend einer der nachfolgenden allgemeinen Formeln:
R¹-[NH-(CH₂)₃]₂-NH₂ ; R¹-[NH-(CH₂)₃]ₙ-NH₂ ;
in welchen die allgemeinen Formeln R¹ und R², identisch oder verschieden, einen C₈₋₂₂-Alkyl- oder -Alkylenrest R bedeuten, wobei der Alkylenrest R 1 oder mehrere ethylenische Doppelbindungen enthält, n eine Zahl im Bereich von 3 bis 6 ist und x, y und z, identisch oder verschieden, Zahlen im Bereich von 1 bis 3 sind.

3. Zusammensetzung nach Anspruch 1 oder 2, dadurch gekennzeichnet, daß der Bestandteil (A) das Salz von einer oder mehreren Carbonfettsäuren mit einem der fetthaltigen Mono-, Di- oder Polyamine ist.

4. Zusammensetzung nach Anspruch 3, dadurch gekennzeichnet, daß das fetthaltige Mono-, Di- oder Polyamin der allgemeinen Formel
R¹-NH-(CH₂)₃-NH₂
entspricht, in welcher R¹ einen C₈₋₂₂-Alkyl- oder -Alkylenrest R bedeutet, wobei der Alkylenrest R eine oder mehrere ethylenische Doppelbindungen enthält.

5. Zusammensetzung nach irgendeinem der Ansprüche 1 bis 4, dadurch gekennzeichnet, daß der Bestandteil (B) das Produkt ist, resultierend aus der Reaktion von einer oder mehreren C₈₋₂₂-Carbonfettsäuren mit Diethylenglykol oder Dipropylenglykol, oder aus der Umesterungsreaktion von einen oder mehreren Glyceriden von C₈₋₂₂-Carbonfettsäuren mit Diethylenglykol oder Dipropylenglykol.

6. Zusammensetzung nach irgendeinem der Ansprüche 1 bis 5, dadurch gekennzeichnet, daß der Bestandteil (B) das Produkt der Umesterungsreaktion von Castoröl mit Diethylenglykol oder Dipropylenglykol ist.

7. Zusammensetzung nach irgendeinem der Ansprüche 1 bis 6, dadurch gekennzeichnet, daß sie von 0,1 bis 1 Gew.-% des Bestandteils (der Bestandteile) (A) und von 1 bis 8 Gew.-% des Bestandteils (der Bestandteile) (B) einschließt.

8. Zusammensetzung nach irgendeinem der Ansprüche 1 bis 7, dadurch gekennzeichnet, daß sie im wesentlichen auf dem Borsäureester von Triethylenglykolmonomethylether basiert und wahlweise einen Glykolether enthält, ausgewählt aus Triethylenglykolmonobutylether oder Monoethylether oder Monomethylether.

9. Verfahren für die Herstellung der Zusammensetzung nach irgendeinem der Ansprüche 1 bis 8, dadurch gekennzeichnet, daß die Bestandteile (A) und (B) und wahlweise andere Bestandteile und Additive mit dem Borsäureester eines Glykolethers unter einer inerten Atmosphäre gemischt sind.

10. Verfahren für die Behandlung einer hydraulischen Flüssigkeitzusammensetzung, einschließend einen Borsäureester eines Glykolethers, um die Korrosion von Eisen(II)-Legierungen oder Metallen in Kontakt mit der erwähnten Zusammensetzung zu reduzieren, einschließend den Zusatz eines korrosionsinhibierenden Systems, dadurch gekennzeichnet, daß das korrosionsinhibierende System einschließt:
(1) Zumindest einen Bestandteil (A), ausgewählt aus fetthaltigen und wahlweise ethoxylierten Mono-, Di- oder Polyaminen, wobei die erwähnten Fettamine zumindest einen C₈₋₂₂-Alkyl- oder -Alkylenrest R enthalten, wobei der Alkylenrest R eine eine oder mehrere ethylenische Doppelbindungen enthalten kann, oder aus den Salzen oder aus einem oder mehreren Carbonsäuren mit den erwähnten Aminen, in einer Menge von 0,05 bis 2 Gew.-% des Bestandteils (der Bestandteile) (A), und
(2) zumindest einen Bestandteil (B), ausgewählt aus den Produkten, resultierend aus der Reaktion von einer oder mehreren Carbonfettsäuren mit einem Polyoxyalkylenglykol, oder aus der Umesterungsreaktion von einem oder mehreren Estern von Carbonfettsäuren mit einem Polyoxyalkylenglykol, in einer Menge von 0,5 bis 10 Gew.-% des Bestandteils (der Bestandteile) (B), wobei die erwähnten Fettsäuren Monocarbonsäuren mit 8 bis 22 Kohlenstoffatomen sind.

## Revendications

1. Composition de fluide hydraulique basée essentiellement sur un ester borique d'un éther de glycol, comprenant un système inhibiteur de corrosion, caractérisée en ce qu'elle comprend :
(1) au moins un constituant (A) choisi parmi des mono-, di- ou polyamines grasses et éventuellement éthoxylées, lesdites amines grasses contenant au moins un radical alkyle ou alkylène C₈-C₂₂ R, le radical alkylène R pouvant contenir une ou plusieurs doubles liaisons éthyléniques, ou parmi des sels d'un ou plusieurs acides carboxyliques avec lesdites amines, à raison de 0,05 à 2% en poids de constituant(s) (A) ; et
(2) au moins un constituant (B) sélectionné parmi les produits résultant de la réaction d'un ou plusieurs acides gras carboxyliques avec un polyoxyalkylène glycol ou de la réaction de transestérification d'un ou plusieurs esters d'acides gras carboxyliques avec un polyoxyalkylène glycol, à raison de 0,5 à 10% en poids de constituant(s) (B), lesdits acides gras étant des acides monocarboxyliques comprenant de 8 à 22 atomes de carbone.

2. Composition selon la revendication 1, caractérisée en ce que le constituant (A) est une mono-, di- ou polyamine grasse correspondant à une des formules générales suivantes :
R¹-NH-(CH₂)₃-NH₂ ; R¹-[NH-(CH₂)₃]₂-NH₂ ; R¹-[NH-(CH₂)₃]ₙ-NH₂
formules générales dans lesquelles, R¹ et R², identiques ou différents, désignent un radical alkyle ou alkylène C₈-C₂₂ R, le radical alkylène R contenant 1 ou plusieurs doubles liaisons éthyléniques, n est un nombre compris entre 3 et 6 et x, y et z, identiques ou différents, sont des nombres compris entre 1 et 3.

3. Composition selon l'une des revendications 1 à 2, caractérisée en ce que le constituant (A) est le sel d'un ou plusieurs acides gras carboxyliques avec l'une parmi les mono-, di- ou polyamines grasses.

4. Composition selon la revendication 3, caractérisée en ce que la mono-, di- ou polyamine grasse correspond à la formule générale
R¹-NH-(CH₂)₃-NH₂
dans laquelle R¹ désigne un radical alkyle ou alkylène C₈-C₂₂ R, le radical alkylène R contenant une ou plusieurs doubles liaisons éthyléniques.

5. Composition selon l'une des revendications 1 à 4, caractérisée en ce que le constituant (B) est le produit résultant de la réaction d'un ou plusieurs acides gras carboxyliques en C₈-C₂₂ avec le diéthylène glycol ou le dipropylène glycol, ou de la réaction de transestérification d'un ou plusieurs esters d'acides gras carboxyliques en C₈-C₂₂ avec le diéthylène glycol ou le dipropylène glycol.

6. Composition selon l'une des revendications 1 à 5, caractérisée en ce que le constituant (B) est le produit résultant de la réaction de transestérification d'huile de ricin avec le diéthylène glycol ou le dipropylène glycol.

7. Composition selon l'une des revendications 1 à 6, caractérisée en ce qu'elle comprend de 0,1 à 1% en poids de constituant(s) (A) et de 1 à 8% en poids de constituant(s) (B) .

8. Composition selon l'une des revendications 1 à 7, caractérisée en ce qu'elle est essentiellement à base d'ester borique de l'éther monométhylique de triéthylène glycol et comprend éventuellement un éther de glycol choisi parmi l'éther monobutylique ou l'éther monoéthylique ou l'éther monométhylique de triéthylène glycol.

9. Procédé pour la préparation de la composition selon l'une des revendications 1 à 8, caractérisé en ce que les constituants (A) et (B) et éventuellement d'autres constituants et additifs sont mélangés avec l'ester borique d'un éther de glycol sous atmosphère inerte.

10. Procédé pour le traitement d'une composition de fluide hydraulique comprenant un ester borique d'un éther de glycol, afin de réduire la corrosion des alliages ou métaux ferreux en contact avec ladite composition, comprenant l'addition d'un système inhibiteur de corrosion, caractérisé en ce que le système inhibiteur de corrosion comprend :
(1) au moins un constituant (A) choisi parmi des mono-, di- ou polyamines grasses et éventuellement éthoxylées, lesdites amines grasses contenant au moins un radical alkyle ou alkylène C₈-C₂₂ R, le radical alkylène R pouvant contenir une ou plusieurs doubles liaisons éthyléniques, ou parmi des sels d'un ou plusieurs acides carboxyliques avec lesdites amines, à raison de 0,05 à 2% en poids de constituant(s) (A) ; et
(2) au moins un constituant (B) choisi parmi les produits résultant de la réaction d'un ou plusieurs acides gras carboxyliques avec un polyoxyalkylène glycol ou de la réaction de transestérification d'un ou plusieurs esters d'acides gras carboxyliques avec un polyoxyalkylène glycol, à raison de 0,5 à 10% en poids de constituant(s) (B), lesdits acides gras étant des acides monocarboxyliques comprenant de 8 à 22 atomes de carbone.
